

M. U. SCHOOP.  
METALLIC COATINGS AND PROCESS OF MAKING SAME.  
APPLICATION FILED APR. 1, 1910.

1,128,058.

Patented Feb. 9, 1915.

2 SHEETS—SHEET 1.

Fig. 1.



Witnesses  
P. Rommers  
E. Leckert.

Inventor  
max Ulrich Schoop  
by *Henry Orthofer*  
Atty

M. U. SCHOOP.

METALLIC COATINGS AND PROCESS OF MAKING SAME.  
APPLICATION FILED APR. 1, 1910.

1,128,058.

Patented Feb. 9, 1915.

2 SHEETS—SHEET 2.

Fig. 1a.



Witnesses

B. Dommer  
E. Leckert.

Inventor  
Max Ulrich Schoop  
by Harry Orth

Attn

# UNITED STATES PATENT OFFICE.

MAX ULRICH SCHOOP, OF HÖNGG, NEAR ZURICH, SWITZERLAND, ASSIGNOR, BY MESNE ASSIGNMENTS, TO METALS COATING COMPANY OF AMERICA, OF BOSTON, MASSACHUSETTS, A CORPORATION OF MASSACHUSETTS.

## METALLIC COATING AND PROCESS OF MAKING SAME.

1,128,058.

Specification of Letters Patent.

Patented Feb. 9, 1915.

Application filed April 1, 1910. Serial No. 552,800.

*To all whom it may concern:*

Be it known that I, MAX ULRICH SCHOOP, a citizen of the Republic of Switzerland, residing at Höngg, near Zurich, Switzerland, have invented certain new and useful Improvements in Metallic Coatings and Processes of Making Same; and I do hereby declare the following to be a full, clear, and exact description of the invention, such as will enable others skilled in the art to which it appertains to make and use the same.

My invention relates to homogeneous metal layers or coatings on articles of various kinds and the process of making same, which coatings may be extremely tenacious, or capable of being removed.

The fundamental idea of the invention consists in that the metal is applied to the surface to be treated, for example articles of metal, wood, paper, fabric and the like, in a finely divided molten or plastic condition, and to this end is sprayed, projected or blown onto the surface to be coated by means of a suitable agent capable of exerting the required pressure, or of atomizing the metal. This agent may be either high pressure steam, hot compressed air, or any other gas or vapor under sufficient pressure to atomize the metal in a suitable atomizer, whether heated or not. Instead of atomizing the metal, the liquid metal may be projected onto the surface to be coated in very fine or capillary streams, or a number of streams united to form a spray, there being used for the purpose one or more nozzles of suitable form through which the molten metal is forced. In some cases I have forced a continuous fine stream of metal from a nozzle and broken the continuity of the stream by rapidly vibrating the nozzle, or a stream of metal may be directed against an inclined plate and thus sprayed. The subdivision of the liquid metal can also be accomplished in a mechanical way by a suitable centrifugal machine, and, finally, a large number of metals may be projected and atomized in a molten state in an apparatus similar in structure to the atomizers used in medicine. The metal in this device is projected or forced from the bath in a fine continuous stream or thread, and then coming into contact with the issuing air or gas is immediately atomized. The pressure medium used for atomizing may be either

neutral, in so far as the metal is concerned, 55 or it may have a chemical action on the metal as it is atomized, which chemical action may be either oxidizing or reducing. It is immaterial how the liquid metal is atomized, or whether the apparatus used 60 for the subdividing the metal as described is stationary or transportable, as the fundamental idea consists in producing coatings of any desired thickness by projecting liquid metal in a finely divided state onto a suitable article or base, said coatings being uniform, homogeneous and of good appearance. If it is important to obtain a coating entirely free, or almost entirely free from 65 oxid, and in case the subdivided or atomized 70 metal has a tendency to oxidize, then it is necessary to use an inert gas as a pressure and atomizing medium. Such a result is, however, not always desired. On the other hand, under certain circumstances it may 75 be advisable to use a gas or vapor having a strong chemical or oxidizing action, thereby obtaining coatings having a more or less predominant metallic appearance, according 80 to the degree of oxidation. However, the same result can be obtained by producing an unoxidized metallic coating in the manner set forth, and subsequently oxidizing the same in an oxidizing atmosphere in a closed 85 chamber, or otherwise. By suitably selecting or dimensioning the atomizing apparatus, the atomized metal can be sub-divided so extremely fine that it resembles a cloud, so that when the article to be coated is brought into the same there results a surface coating having a beautiful, smooth metallic luster. The metallic microscopic globules or drops of this metallic cloud, on account of their great speed, due to the liquid metal being under pressure, are projected with great force from the atomizing nozzle. These globules are flattened out 90 and formed into very thin scales that lie adjacent to and overlap one another, so that they are welded together, which results in 100 an intimately connected metallic sheet or coherent metallic body whose structure is very dense and tough.

This coating may be composed of a mixture of metals, by using a molten mixture 105 which is atomized and projected onto the body or article to be coated. Fluxes may be used, and added to the metal in the melting

pot, and the flux may be such that it is vaporized and produces the vapor that gives the required pressure for the atomization of the molten metal. Admixtures of metals 5 may be used. Various vapors or gases may be used to produce the atomization of the metal at the atomizing nozzle whose chemical action on the metal will change the appearance of the coating. The structure and 10 chemical character of the finished metal coating is, therefore, dependent upon the manner in which it is produced, and must be varied according to the effect to be achieved on the article to be coated.

15 Coatings may be made that may be subjected to any desired subsequent mechanical treatment, such as pressing, stamping, dressing, planing, etc., without damaging them or loosening them from their bases.

20 The melting point of the metal of the coating, the character and temperature of the surface to be coated, the pressure used in atomizing and the thickness to be attained, as well as the distance of the nozzle from the 25 object to be coated, will more or less influence the character of the coatings to be made as well as the manner in which the coatings are made. It is sometimes advisable to subject the objects to be coated to a certain cleaning 30 action, for example, to clean them by a sand blast from adhering dirt, oxid, or the like, or by means of an acid or any other substance used for cleaning metal surfaces; further, in many cases it is advantageous, 35 especially where metallic articles are to be coated or plated to meet varying demands of trade, to heat these articles before or during the coating operation, and thereby insure a coating that will strongly adhere to 40 its base.

Nearly all metals are sufficiently fluid at suitable temperatures to produce fine subdivision in accordance with this invention, and no difficulty is found in working with 45 them. Some metals, however, present difficulties, such as zinc and aluminium, which can only be sub-divided or atomized by mixing them with fluxes or with other metals in small quantities. By this process it is possible to produce durable aluminium articles 50 in a practical manner, or to coat metallic articles with aluminium, which has heretofore not been possible electrolytically.

55 It is obvious that alloys of metals may be used instead of substantially pure metals.

Thus far I have described the making of coatings which strongly adhere to their bases, but my invention is not limited to such coatings.

60 I will now describe how I make removable metal coatings, for the reproduction of printing clichés, medals, &c. In order to produce these removable coatings it is necessary or advisable to oil or grease the matrix or base, to coat it with graphite, or

treat it in any other well-known manner for the purpose of preventing the adhesion of the metallic coating; and in some cases it is desirable to keep the matrix heated during the application of the metallic coating, but this may be dispensed with in the majority of cases where the coating to be applied is not extraordinarily thick. In order to make a comparatively thick coating, and thereby a coating readily separable from its base, 70 the time, during which the surface from which the impression is to be taken is exposed to the atomized or finely divided metal, is regulated in accordance with the thickness of the reproduction to be obtained. For example, for the manufacture of printing clichés of about six millimeters thickness, it is generally sufficient to expose the negative mold to the action of the atomized metal for about ten seconds. After the 75 metallic coating has been formed on the matrix as above described, the matrix may be dropped into cold water to quickly shrink it, and thereby readily release it from the article made.

80 In certain cases it is quite possible to make extremely thin metal sheets, that are readily removed from their bases, for example, for the production of metallic foil; and in some instances it is advisable to have the matrix 85 or base as smooth as possible, in order to more readily release the metal coating after it has been formed.

90 Metallic sheets or foils which have been formed on polished or cut glass in the manner described, will adhere to these only by the action of atmospheric pressure, and remind one in their structure and general appearance of the photographic transfers made on polished glass, and have a very high 95 luster.

100 By my method it is possible to quickly and cheaply reproduce matrices and printing blocks of all kinds, medallions, and the like, which has heretofore been done by electrolytic methods. In ten hours, with the same negative matrix, from three hundred to four hundred reproductions can be made, which are as sharp and fine in every detail, and as beautiful in their appearance 105 as electrically plated reproductions. The metallic particles are thrown with great force, compared to their size, onto the matrix or support, and are cemented or welded together into a compact metallic sheet forming a coherent metallic body. A further 110 advantage of my new process consists in that the electrolytic bath is entirely avoided, so that bodies of any desired shape and size may be reproduced, hollow bodies being 115 made in parts which are afterward soldered together, and any metal whatever may be used to reproduce these articles, so that aluminium and other metals can be used, 120 which cannot readily be done in an electro- 125

lytic bath. Further, it is readily possible to make seamless metallic tubes, or hollow vessels, and to this end a core of suitable material is placed in the metallic cloud and rotated, or the atomizer may be moved around the core or base to be covered; after which the core is either physically or chemically removed, by melting or burning it out, or by removing it by acids. The thickness 5 of these removable metal coatings may be varied within comparatively wide limits, and the thickness obtained within a definite time will depend upon the gas pressure used for atomizing or subdividing the liquid 10 metal, and upon the gas itself, whether oxidizing, reducing or neutral. The distance the object is held from the atomizing nozzle, as well as the size of the openings in said atomizing nozzle are also factors upon which 15 the thickness depends. The density of the particles of coating is dependent upon the distance the article is held from the atomizing nozzle, as the shorter the distance the less time the atomized particles have to cool 20 or set, or to become oxidized. If the pressure medium used for atomizing the fluid metal is neutral, then there is practically no difference whatever in the metallic coating 25 formed and the general character of the metal. If the pressure medium is capable 30 of oxidizing the metal, then the coating contains more or less oxid and is more or less porous, so that there will be a limitation to the thickness to which said coating can 35 be made.

A peculiarity of the metallic cloud, or atomized metal, is that in general its temperature is very low, and the finer the atomization the lower the temperature, and 40 of course the finer the atomization the greater will have to be the gas pressure used to produce it, so that materials may be used as matrices whose melting and ignition temperatures are very low, for example, such materials as hard paper and celluloid. It is also possible to hold the naked hand in the metallic cloud without 45 injury, or without feeling any pain, which shows that the most delicate tissues can be reproduced. The temperature may be varied 50 within wide limits as circumstances demand or permit. I have used the process in cases where the temperature of the metallic cloud was in the neighborhood of 60° Celsius, and 55 also in cases where the temperature was increased to 200° Celsius and more.

Figures 1 and 1<sup>a</sup> taken together show by way of example one form of apparatus suitable for carrying out my invention, being 60 partly in section and partly in elevation.

In the particular form of apparatus illustrated, *a*, *a*, are the steel flasks containing compressed gas, for example, air. These flasks are connected to a coil *c* contained in 65 a suitable casing *c'* provided with a gas

burner *d* for heating the coil and the air therein which has become cold by reason of expansion. The metal *f* is contained in a preferably but not necessarily closed melting pot *i* provided with a valve *h* controlling the outlet to the pipe *m* which terminates in a downwardly directed nozzle *g*. The heating coil *c* has two branches, one *k* entering the pot *i* above the level of the metal *f* and the other *l* terminating adjacent the 70 nozzle *g*. The atomized metal is directed onto the object *e* to be coated, which is contained in a chamber *n*. Pressure gages *b*, *b* are placed in the gas conduit.

I claim—

1. The process of metallically plating or coating articles, which comprises finely and uniformly subdividing a molten metal maintained under pressure, and projecting it upon the surface to be coated with sufficient 85 force to produce a uniform, non-porous welded coating.

2. The process of forming a coherent metallic body, which comprises finely subdividing a metal under the combined action of 90 heat and pressure, and substantially at the same time projecting said subdivisions upon a surface with sufficient force to produce a non-porous, homogeneous body.

3. The process of forming a coherent metallic body, which comprises finely subdividing a metal under the combined action of 95 heat and pressure, and substantially at the same time projecting said subdivisions upon a surface with sufficient force to produce a 100 non-porous, homogeneous body, and controlling the pressure during projection.

4. The process of metallically plating or coating articles, which comprises finely and uniformly subdividing a molten metal by 105 means of a gaseous pressure medium having a coloring action on the metal and projecting the finely divided metal by the same medium upon the surface to be coated with sufficient force to produce a non-porous 110 welded coating.

5. The process of metallically plating or coating articles, which comprises finely and uniformly subdividing a molten metal under pressure, and projecting the finely divided 115 molten metal onto the surface to be coated, by means of a gas capable of acting chemically on the metal.

6. The process of metallically plating or coating articles, which comprises atomizing a molten metal by means of a gas capable of oxidizing the metal to be atomized, and projecting the finely divided metal upon the 120 surfaces to be coated.

7. The process of metallically plating or coating articles, which comprises providing the articles with a clean surface and projecting atomized liquid metal under pressure onto the articles.

8. The process of metallically plating or 130

coating articles, which comprises cleaning the articles and projecting atomized liquid metal onto the article while hot with a force sufficient to flatten the particles of metal and thereby weld them into a uniform non-porous coating.

9. An article having a metallic coating, said coating comprising finely divided metallic particles of uniform size adjacent to 10 and overlapping one another in a non-porous coating of uniform surface texture.

10. An article having a metallic coating, said coating comprising finely divided, more or less flattened metallic globules adjacent 15 to and overlapping one another and welded together, presenting a uniform, non-porous surface readily burnished.

11. The process of metallically plating or coating articles, which comprises finely and 20 uniformly dividing molten metal under pressure, and projecting the finely and uniformly divided metal upon the article to be coated while said article is heated.

12. The process of forming a coherent 25 metallic body, which comprises finely subdividing a metal under the combined action of heat and pressure, and substantially at the same time projecting said subdivisions while exerting a chemical action thereon, 30 upon a surface with sufficient force to produce a non-porous, homogeneous body.

13. The process of forming a coherent metallic body, which comprises finely subdividing a metal under the combined action of 35 heat and pressure, and substantially at the same time projecting said subdivisions by a gaseous medium upon a surface with sufficient force to produce a non-porous, homogeneous coating and controlling the pressure 40 of said medium.

14. The process of forming a coherent metallic body, which consists in finely subdividing a metal under the combined action of heat and a gaseous pressure medium having 45 a coloring action on the metal, and substantially at the same time projecting said subdivisions upon a surface with sufficient force to produce a non-porous, homogeneous body.

50 15. The process of forming a coherent metallic body, which consists in finely subdividing a metal under the combined action

of heat and a gaseous pressure medium having a coloring action on the metal, and substantially at the same time projecting said 55 subdivisions upon a surface with sufficient force to produce a non-porous, homogeneous body, and controlling the pressure of said medium.

16. The process of forming a coherent 60 metallic body, which consists in finely subdividing a metal under the combined action of heat and a gaseous pressure medium having a chemical action on the metal, and substantially at the same time projecting said 65 subdivisions upon a surface with sufficient force to produce a non-porous, homogeneous body.

17. The process of forming a coherent metallic body, which consists in finely sub-dividing a metal under the combined action of heat and a gaseous pressure medium having a chemical action on the metal, and substantially at the same time projecting said subdivisions upon a surface with sufficient force 75 to produce a non-porous, homogeneous body, and controlling the pressure of said medium.

18. The process of forming a coherent metallic body, which consists in finely sub-dividing a metal under the combined action 80 of heat and a gaseous pressure medium capable of oxidizing the metal, and substantially at the same time projecting said subdivisions upon a surface with sufficient force to produce a partially oxidized, non-porous, 85 homogeneous body.

19. The process of forming a coherent metallic body, which consists in finely sub-dividing a metal under the combined action of heat and a gaseous pressure medium capable of oxidizing the metal, and substantially at the same time projecting said subdivisions upon a surface with sufficient force to produce a partially oxidized, non-porous, 90 homogeneous body, and controlling the pressure of said medium.

In testimony that I claim the foregoing as my invention, I have signed my name in presence of two subscribing witnesses.

MAX ULRICH SCHOOP.

Witnesses:

WILHELM REINHARD,  
CARL GUBLER.